# EUROPEAN PATENT APPLICATION

(11) **EP 1 126 545 A1**
(43) Date of publication of application: **22.08.2001**
(21) Application number: 00870020.5
(22) Date of filing: 14.02.2000
(51) Int. Cl.: H01Q 15/08, H01B 3/44, H01B 3/00

(54) **Dielectric material composition**

(71) Applicant: Emerson & Cuming Microwave Products, 2260 Westerlo (BE)
(72) Inventor: Schryvers, Joris, 2140 Antwerpen (BE); Timmerman, August, 2260 Westerlo (BE); Van Roy, Petrus, 3290 Diest (BE)
(74) Representative: Luys, Marie-José A.H.

(57) **Abstract**

The present invention relates to a dielectric material composition containing particles of a plastic material and an amount of a titanium-oxygen compound, wherein the plastic material is an expandable plastic material and in that the particles of the plastic material are coated with a coating of the titanium-oxygen compound.

## Description

The present invention relates to a dielectric material composition as described in the preamble of the first claim.

Dielectric materials find numerous applications, e.g. in printed circuit boards, in lens antennas and passive reflectors as is disclosed in Electronic Design, April 13, 1960 by E.F. Buckley "Stepped-index Luneberg lenses: antennas and reflective devices." By placing a small and broad beamed feed antenna with its effective phase centre at the focal radius of the lens, an efficient lens antenna results because all energy radiated into the forward hemisphere is theoretically collimated. By covering a portion of the surface of the lens with a metallic reflector, the combination of the reflector and the lens serves as a passive reflector of microwave energy throughout a solid angle equal to that subtended by the reflector.

Luneberg lenses are mostly spherical symmetric lenses that are built up of a plurality of individual lens shells that fit into each other to form a sphere of pre-determined dimensions. The geometry of the lens is namely dictated by the frequency of the radiation involved. The focusing properties of such a lens are defined by the relationship dielectric constant - radius of the spherical shells. Ideally, the relationship between the relative dielectric constant *k* and radius *r* of the individual shells is:$\text{k} \text{=} \text{2} \text{-} {\text{r}}^{\text{2}} \text{formula I}$ in the range 0 r 1. In general, it is required that the variation of the relative dielectric constant is between 1 at the surface of the spherical lens and 2 at the centre.

To achieve a smooth variation of the dielectric constant from the centre towards the lens surface, lenses have been made in which a series of circular shells of different radii are fit into one another to approximate a sphere. To reduce the dielectric constant k to the correct value at each point in the sphere, holes are drilled in each shell. Such shells however are neither homogeneous nor isotropic. In another solution the lens is made of foamed plastic materials the density of which is varied to reduce the dielectric constant k to the correct value at each point in the sphere. In that way a stepwise approximation to formula I defining the relation between k and r, can be achieved. An optimal approximation to the theoretical smooth curve of k can be achieved if the number of shells is as large as possible. Economy of fabrication however dictates to keep the number of shells required as low as possible.

To allow k to be further varied, use has been made of dielectric material compositions in which a high-k material, such as titanium dioxide is dispersed as a powder in a low-k material, usually a powder of a plastic material. After dispersion of the titaniumdioxide in the plastic material the composition is subjected to a foaming step, so as to achieve the desired density. However, these compositions have not been widely employed in Luneberg lenses.

One of the reasons is that because of the relatively large difference between the density of the plastic material and the titanium dioxide, the distribution of the titaniumdioxide in the plastic material is insufficiently homogeneous as a consequence of which within a shell made of such a material will show a non-uniform dielectric constant.

It is the aim of the present invention to provide a dielectric material composition with an improved homogeneity.

This is achieved with the present invention with the features of the characterising part of the first claim.

By applying the titanium-oxygen compound containing composition as a coating to the plastic material in stead of mixing it therewith, a more uniform distribution of the composition over the plastic material particles can be achieved. This in turn allows a lens with a more homogeneous lens behaviour to be obtained.

Depending on the nature of the plastic material, it may have a relatively low k value, whereas the k of titanium-oxygen compounds is significantly higher. As a consequence, a relatively small amount of the titanium-oxygen compound suffices to increase the k value of the composition, so that the density of the composition and consequently the density and weight of a lens made of such composition can be kept low. This is important in modern applications of the composition, for example in antennas where severe restrictions with respect to the weight of the antenna are imposed by law, while simultaneously the material the antenna is made of should have at least a pre-determined k so as to allow the antenna to be used for its application. To keep the density and thus the weight of the composition as low as possible, the composition preferably contains an expandable plastic material.

In the composition of this invention use can be made of the titanium oxide compounds that are generally known to the man skilled in the art. Examples of suitable titanium-oxygen compounds include titaniumdioxide, bariumtitanate BaTiO₃, strontiumtitanate SrTiO₃, but other titanium-oxide compounds may be used. Preferably use is made of titaniumdioxide because of its high k value which may vary from approximately 80 to approximately 100, combined with a low dissipation factor (low dielectric losses), a relatively low density of approximately 3.8 - 4.3, good stability as a function of temperature of the dielectric behaviour and because it is easily commercially available. The use of titaniumdioxide allows a lens to be obtained with a relatively low weight at high k-value and low dissipation losses.

Besides titanium-oxygen compounds, also other compounds with a suitable dielectric constant may be used contained in the coating. Possible examples include ceramic powders, for example silicondioxide, siliconcarbide, siliconnitride, magnesiumoxide etc.

Titaniumdioxide is preferably added in an amount of 5-65 % by weight with respect to the total weight of the composition. Below this range the volume of the titaniumoxide used gets small, which on the one hand may result in a coating with an insufficient homogeneity and on the other hand affect the k-value to only a small or negligible extent. Above this range there is a risk to a decreasing adhesion of titanium oxide to the plastic material. Simultaneously, the presence of the coating counteracts expansion of the plastic material in case use is made of non or partly expanded plastic material thus counteracting that the density aimed at can be obtained. Care should be taken to find the optimum compromise between allowing a sufficient expansion to take place and obtaining a composition with the desired k value.

The mean particle size of the titanium-oxygen compound coating is preferably maintained within well defined range so as to allow an optimum and uniform coating to be obtained. Thereto, the mean particle size is preferably smaller than 50*µ*m, more preferably smaller than 10*µ*m.

The plastic material used in the composition of the present invention further preferably comprises an expandable plastic material. Suitable plastic materials include expandable plastic materials generally known to the man skilled in the art, for example homopolymers or copolymers of polypropylene, polyethylene, ABS, polyvinylchloride, polystyrene etc. Polystyrene is preferred over the other materials because of its excellent dimensional stability in the sense that the shrink after expansion is limited. This is important in case the material is expanded while moulding it into a part for example a lens part, of a pre-determined shape and pre-determined dimensions. In Luneberg lenses namely, parts of increasing dimensions have to fit closely to each other to allow a spherical lens to be obtained. Polystyrene further has a relatively low density combined with low dissipation losses.

The polystyrene used in the composition of this invention may be partly or completely pre-expanded, so as to provide particles with a larger volume and to allow the titanium-oxygen coating to be applied in an optimum manner. Whereas a non-expanded polystyrene for example may have a material density of approximately 1050 g/l and a bulk density of 600-700 g/l, the bulk density of expanded polystyrene may be decreased to 10-300 g/l, preferably 60-300 g/l depending on the degree of expansion, but is preferably at least 60 g/l. However, polystyrene particles with lower or higher densities may be used, the maximum possible density corresponding to the density of unexpanded polystyrene, the density preferably being at least 60 g/l.

From US-A-4.288.337 a dielectric composition is known wherein expanded polystyrene particles are coated with a metal film. Mixing such coated particles with untreated expanded polystyrene may lead to the desired dielectric constant. Such a process however involves an additional process step as both coated and uncoated particles need to be mixed. In order to achieve a homogeneous mixing, it is adviseable that the coated and uncoated plastic material particles have approximately the same density. Furthermore, since metal-metal contacts have to be avoided as they give rise to undesired dielectric losses, the amount of metal coated particles the can be incorporated in the mixture, is limited. As a consequence, the range of dielectric constants that can be achieved with such a mixture is limited. Finally, it is adviseable to add a binder material to optimise the adhesion between the metal coated and the non coated particles. This again involves an additional process step.

To improve the binding of the titanium-oxygen compound coating on the particulate plastic material, the composition preferably contains an apolar adhesive or binder, for example a wax, a polyurethane resin or an epoxy resin. The use of an apolar binder allows to minimise the dissipation factor. The binder is preferably used in an amount of 1-25 percent by weight of solid binder with respect to the total weight of the composition. The volume ratio of the binder with respect to the titanium-oxygen compound is preferably at least 1/4 in order to allow the titanium-oxygen compound to be sufficiently captured in the binder material.

With the present invention, dielectric materials can be obtained which have a bulk density that may vary from approximately 150 to approximately 700 g/l, a dielectric constant of between approximately 1.2 - 10, preferably 1.2 - 5 and dielectric losses of below approximately 0.005. The latter is important as it adversely affects the functioning of the lens. Up to now materials that simultaneously show a low density, high *k* and low dielectric losses had not been available.

The present invention also relates to parts, in particular a lens or an antenna made of a material comprising the dielectric composition of this invention.

In a process for producing parts comprising the material of this invention, preferably the plastic material particles are mixed with the binder, whereafter the titanium-oxygen compound is added. The binder is preferably applied as a binder emulsion so as to allow a uniform application to be achieved. After having been thoroughly mixed, the composition can be moulded in a mould at a predetermined temperature and pressure. As a plastic material, either an unexpanded or a partly expanded material can be used, depending on the density of the final product aimed at. The use of unexpanded or partly expanded material allows to avoid the formation of gas inclusions in the moulded part. The density of the final product can be further controlled by controlling the moulding temperature, as this determines the expansion of the plastic material. Often, steam is blown into the mould to cause expansion of the plastic material. After the plastic material has expanded to the desired extent, vacuum is applied so as to remove the excess of foaming agent and water from the mould as the former may affect the dimensional stability of the moulded part, whereas the latter may adversely affect the dielectric properties of the material. Finally, the moulded part is subjected to a drying step to remove any remaining water.

The invention is further illustrated in the following examples.

### Example 1.

35 parts by weight of expanded polystyrene homopolymer with a density of 150 g/l were mixed with 20 parts by weight of a water diluted wax solution which contained 15 parts of solid wax. Then, 45 parts by weight of TiO₂ were added so as to obtain an optimal wetting of the TiO₂. The mixture was moved during a sufficiently long period to ensure that all particles are well wetted and that the excess of water present in the wax emulsion is evaporated.

After the particles had been coated with TiO₂, an amount of the coated particles was introduced into a mould and moulded into a part. The mould was closed and heated to 100°C by immersion in boiling water. After approximately 15 minutes, the moulded part was removed from the mould and allowed to dry at 70°C for 10 hours.

The part was characterised by determining the dielectric properties or permittivity of the material. The real part of the permittivity between 8 and 12.5 Ghz (X-band) is shown in figure 1, the imaginary part is shown in figure 2.

### Example 2.

Additional compositions were prepared as described in Example 1, except that the amount of filler and/or binder was varied as given in table 1. Table 1 also gives the variation of k as a function of the density of the composition. As can be seen from figure 3, compositions with a density of up to 400 g/l can be obtained at dielectric constants as high as 1.8. By further varying the density of the polystyrene particles and the amount of wax and/or titaniumdioxide, compositions can be made with even a higher dielectric constant for example up to 2.2 and a density of about 600 g/l. Dielectric losses of the various materials were below 0.005.

The range of density/dielectric constant combinations that can be achieved with a polystyrene, TiO₂ composition is shown by the solid lines A, B in figure 3. This range is mainly determined by the degree of pre-expansion of the polystyrene particles.

**Table 1:**

| Compositions as mixed. | | | | | |
|---|---|---|---|---|---|
| Sample n° | 1 | 2 | 3 | 4 | 5 |
| EPS (parts by weight) | 50 | 35.0 | 25 | 65 | 67.1 |
| Wax emulsion, 15 parts by weight of solid wax | 14.2 | 20.0 | - | 17.5 | - |
| Wax emulsion, 60 parts by weight of solid wax | - | - | 25.0 | - | 11 |
| TiO₂ | 35.7 | 45.0 | 50.0 | 17.5 | 21.9 |
| Density | 294 | 330 | 492 | 642 | 550 |
| Permittivity | 1.5 | 1.7 | 2.5 | 2.6 | 2.75 |

**Table 2:**

| Compositions as dried. | | | | | |
|---|---|---|---|---|---|
| Sample n° | 1 | 2 | 3 | 4 | 5 |
| EPS (parts by weight) | 56.9 | 42.2 | 27.8 | 79.3 | 70.2 |
| Solid wax | 2.4 | 3.6 | 16.7 | 3.15 | 6.9 |
| TiO₂ | 40.7 | 54.2 | 55.5 | 20.6 | 22.9 |
| Density | 294 | 330 | 492 | 642 | 550 |
| Permittivity | 1.5 | 1.7 | 2.5 | 2.6 | 2.75 |

## Claims

1. A dielectric material composition containing particles of a plastic material and an amount of a titanium-oxygen compound, characterised in that the plastic material is an expandable plastic material and in that the particles of the plastic material are coated with a coating of the titanium-oxygen compound.

2. A dielectric material composition as claimed in claim 1, characterised in that the titanium-oxygen compound is titanium dioxide.

3. A dielectric material composition as claimed in any one of claims 1 or 2, characterised in that the composition comprises 5-65 wt. % of the titanium-oxygen compound with respect to the total weight of the material.

4. A dielectric material composition as claimed in any one of claims 1-3, characterised in that the composition comprises 1-25 % by weight of a solid binder with respect to the total weight of the composition.

5. A dielectric material composition as claimed in any one of claims 1-4, characterised in that the expandable plastic material is polystyrene.

6. A dielectric material composition as claimed in claim 5, characterised in that the expanded polystyrene has a density of at least 60 g/l.

7. A sphere or hemispherical shell comprising a composition as claimed in any one of claims 1-6.
